# EUROPEAN PATENT SPECIFICATION

(11) **EP 2 578 666 B1**
(45) Date of publication and mention of the grant of the patent: **15.11.2017**
(21) Application number: 10852594.0
(22) Date of filing: 28.12.2010
(51) Int. Cl.: C10B 55/00, C10G 9/00, C10B 57/04

(54) **METHOD FOR PRODUCING A COKING ADDITIVE BY DELAYED COKING**
VERFAHREN ZUR HERSTELLUNG EINES KOKUNGSZUSATZES MITTELS VERZÖGERTER VERKOKUNG
PROCESSUS DE PRODUCTION D'ADDITIF DE COKÉFACTION PAR COKÉFACTION LENTE

(30) Priority: 01.06.2010 RU 2010122135
(43) Date of publication of application: 10.04.2013
(73) Proprietor: Obshhestvo S Ogranichennoi Otvetstvennost'yu "Promintekh", Perm 614000 (RU)
(72) Inventor: VALYAVIN, Gennady Georgievich, Ufa 450055 (RU); VETOSHKIN, Nikolai Ivanovich, Ufa 450061 (RU); ZAPORIN, Victor Pavlovich, Ufa 450068 (RU); SUKHOV, Sergei Vital'evich, Ufa 450007 (RU); MAMAEV, Mikhail Vladimirovich, Perm 614030 (RU); BIDILO, Igor Viktorovich, Ufa 450075 (RU); VALYAVIN, Konstantin Gennad'evich, Ufa 450055 (RU); STUKOV, Mikhail Ivanovich, Ekaterinburg 620049 (RU); ZAGAINOV, Vladimir Semenovich, Ekaterinburg 620149 (RU)
(74) Representative: Spengler, Robert
(86) International application number: PCT/RU2010/000795
(87) International publication number: WO 2011/152752

(56) References cited:
- JP-A- 2008 063 529
- RU-C1- 2 067 605
- RU-C1- 2 206 595
- US-A- 4 036 736
- US-A- 5 028 311

## Description

This invention relates to oil refining, in particular to delayed coking that produces coke containing 15-25% of volatiles substances, which can be used as a coking additive in a coal coking charge for metallurgical coke production.

Oil coke with more than 14% but less than 25% volatiles is capable not only of replacing the K-brand (coking) coal, which is in short supply, in coal coking charges, but also of improving the quality of metallurgical coke (Russian Federation Patent 2355729, C10B57/04, published on 20 May 2009).

There exists technology for forming oil coke by delayed coking of oil residues. This method includes slowly heating raw materials to 490-515°C in a tubular furnace, mixing the raw materials with a recirculant, presenting the coking distillate products formed inside the coking chamber, in a rectification column, which produces bottoms, supplying the bottoms as the secondary raw materials to the coking chamber at 485-495°C and carrying out coking, which results in the formation of coke (Z. I. Syunyaev, "Forming, Refining and Using Petroleum Coke", Moscow: Khimiya: 1973, p. 95).

The drawback of this method is that the coke formed by its application has a high strength and low concentration of volatiles (up to 9% by mass).

It is possible to increase the concentration of volatiles in coke by reducing the temperature of the raw materials at the inlet into the coking chamber. However, reducing that temperature and coking at low temperatures results in excessive foaming and, consequently, it increases the probability of the foam getting into the rectification column, then into the furnace, which might result in the plant becoming coked up, shortening the spans between overhauls.

A delayed coking method, capable of guaranteeing that no direct contact would occur between the primary charge and the vapours reaching the rectification column from the coking chamber during the formation of the secondary charge, can prevent coke foam finding its way inside the reaction spiral tubes of the furnace, the coking up of the plant and thus lengthen the spans between overhauls.

The technology nearest to the proposed invention is the delayed coking of oil residues, which includes heating the original raw materials to 340-380°C, mixing them with a recirculant- heavy coking gasoil (pyrolisis resin, heavy catalytic cracking gasoil)- in a mixing tank where the secondary charge forms, heating the secondary charge, i.e. the heavy residues formed in the mixing tank, transferring this into the coking chamber at 485-505°C, and coking to form coke (Russian Federation Patent No. 2206595, class C10B 55/00, published on 20 June 2003).

The drawback of this invention is the low concentration of volatiles in the final product due to the high coking temperature (485-505°C) and the low efficiency due to extensive foaming, and consequently to not being able to use the coking chamber to its full capacity.

This invention aims at increasing the concentration of volatiles in the coke and improving the efficiency of the plant.

This aim is achieved because this method of delayed coking of a coking additive includes preheating of the primary raw materials at 270-350°C, and in particular at 270-330°C, mixing the primary raw materials with the recirculant in the tank for the production of secondary charge, heating the secondary charge, transporting it to the coking chamber, and coking to form the target product. In this invention the secondary charge is heated at 455-470°C before it reaches the coking chamber.

Moreover, to prevent foaming, an anti-foaming dope is introduced into the coking chamber 3-5 hours before the end of coking.

Moreover, taking into consideration that the foam developed in low-temperature coking forms a thick layer, the anti-foaming dope is introduced in two to four areas around the perimeter of the coking chamber, so that it covers the entire surface of the foam.

Coking carried out at low temperatures, because the raw material is charged into the coking chamber at a low temperature, produces coke with a concentration of volatiles of 15-25% to be used as a coking additive.

Introducing the anti-foaming dope during the last 3-5 hours of the coking process not only reduces the amount of foam forming in the coking chamber but also makes the process more efficient with respect to the primary raw materials.

The diagram shows the main parts of the plant for carrying out the proposed method for production of a coking additive by the means of delayed coking.

The proposed method of production of a coking additive in delayed coking works as follows.

The original raw materials, such as tar, de-asphalting asphalt, oil production extracts, heavy gasoil of catalytic cracking or any mixtures of the above, are heated in a tubular furnace 1 to 270-350°C, and in particular to 270-330°C, then discharged into the mixing tank 2 connected in pairs to the rectification column 3. Heavy coking gasoil, used as the recirculant, is also charged from the rectification column 3 as a side fraction.

The mixture of the primary raw materials and recirculant, which becomes the secondary charge, is heated to 455-470°C in the tubular furnace 4, then fed into the alternately working coking chambers 5 where a coking additive with 15-25% volatiles is gradually accumulated. The distillate coking products, formed in the coking chamber 5, are discharged into the rectification column 3, where they are resolved into a gas, benzene, light and heavy coking gasoil and the bottoms.

Vapour-like products leave the plant through the top of the column 3, light and heavy gasoils are discharged from the middle part of the column, while the bottoms are removed from the bottom part. To reduce foam formation, 3-5 hours before the end of coking, the anti-foaming dope is introduced in four areas around the perimeter of the coking chamber 5.

The suggested technology is illustrated with the following four examples: 1-4.

A mixture of raw materials, comprised of a vacuum visbreaking residue, tar oil and heavy gasoil of catalytic cracking in the ratio of 15:75:10 was coked, using an industrial delayed coking plant. The mixture had the following characteristics: density 1.055 g/cm³, cokeability 25.8% and sulphur content 3.8%. The primary charge was heated in a convection furnace to 320°C, then it was mixed with a recirculate: heavy coking gasoil, discharged from the rectification column as a side fraction. The produced secondary charge was heated in a tubular furnace, then it was fed into the coking chamber to produce a coking additive. When coking was over, the coke was steamed out, water-cooled and discharged by hydraulic means. In Examples 2 and 4, an anti-foaming dope was introduced into the coking chamber 4 hours before the end of the process - to prevent foam formation.

Coking conditions and results in Examples 1-4 are shown in the Table.

For comparison, the same charge as in 1-4 was coked, using the technology of the prototype of this invention. The temperature of the secondary charge at the inlet of the coking chamber was 485°C. No anti-foaming dope was used. The result was ordinary electrode coke with a concentration of volatiles of 10.8%. The conditions and results are also presented in the Table.

**Table**

| Comparative Data on Coking of Raw Materials | | | | | |
|---|---|---|---|---|---|
| Characteristics | Example | | | | |
| | Invention technology | | | | Prototype |
| | 1 | 2 | 3 | 4 | 5 |
| Plant efficiency with respect to primary charge, m³/h | 96 | 100 | 96 | 98 | 95 |
| Plant efficiency respective the secondary charge, m³/h | 106 | 110 | 110 | 112 | 105 |
| Secondary charge temperature at the coking chamber inlet, °C | 468 | 468 | 456 | 456 | 485 |
| Coking duration, h | 16 | 16 | 16 | 16 | 16 |
| Coke level in the chamber, m | 19.0 | 20,5 | 19.5 | 21.0 | 19.0 |
| Concentration of volatiles in coke, % | 15.1 | 15.5 | 21.8 | 22.4 | 10.8 |
| Anti-foam ing dope, yes/no | No | Yes | No | Yes | No |

As can be seen from the Table, the coking method suggested by this inventor produces coke that can be used as a coking additive, with a concentration of volatiles higher than 15%. Introducing it into the coking chamber below 456°C is not practicable because bitumen is likely to form, and it would make the steaming out and cooling down of coke difficult. On the other hand, a charge introduced at a temperature above 470°C, will produce coke that contains less than 15% of volatiles.

Introduction of the anti-foam dope into the top part of the coking chamber reduces the amount of foam that forms during coking, which improves the working efficiency of this technology with respect to the original raw material.

## Claims

1. A method of producing a coking additive in delayed coking, which includes heating the primary charge to 270-350°C, mixing the primary charge with a recirculate in a tank, which makes a secondary charge, heating the secondary charge and introducing it into the coking chamber, coking to form the target product, different in that the secondary charge is introduced into the coking chamber at 455-470°C.

2. A method as in 1, different in that an anti-foaming dope is introduced into the coke chamber 3-5 hours before the end of coking.

3. A method as in 1, different in that the anti-foaming dope is introduced into 2-4 areas around the perimeter of the coking chamber.

## Patentansprüche

1. Verfahren zur Herstellung eines Verkokungshilfsmittels bei verzögerter Verkokung, das umfasst: Erhitzen der Primärladung auf 270 bis 350 °C, Mischen der Primärladung mit einem Rezirkulat in einem Tank, was eine Sekundärladung ergibt, Erhitzen der Sekundärladung und Einführen derselben in die Verkokungskammer, Verkoken, um das Zielprodukt zu bilden, sich dadurch unterscheidend, dass die Sekundärladung bei 455 bis 470 °C in die Verkokungskammer eingeführt wird.

2. Verfahren nach Anspruch 1, sich dadurch unterscheidend, dass 3 bis 5 Stunden vor dem Ende der Verkokung ein Antischaumadditiv in die Verkokungskammer eingeführt wird.

3. Verfahren nach Anspruch 1, sich dadurch unterscheidend, dass das Antischaumadditiv in bis 2 bis 4 Bereiche um den Umfang der Verkokungskammer eingeführt wird.

## Revendications

1. Procédé de production d'un additif de cokéfaction par cokéfaction lente, qui comprend le chauffage de la charge primaire à une température de 270 à 350 °C, le mélange de la charge primaire avec une substance recyclée dans un réservoir, pour obtenir une charge secondaire, le chauffage de la charge secondaire et l'introduction de celle-ci dans la chambre de cokéfaction, la cokéfaction pour former le produit cible, différent en ce que la charge secondaire est introduite dans la chambre de cokéfaction à une température de 455 à 470 °C.

2. Procédé selon la revendication 1, différent en ce qu'un dopant anti-mousse est introduit dans la chambre de cokéfaction 3 à 5 heures avant la fin de la cokéfaction.

3. Procédé selon la revendication 1, différent en ce que le dopant anti-mousse est introduit dans 2 à 4 zones autour du périmètre de la chambre de cokéfaction.
